# EUROPEAN PATENT APPLICATION

(11) **EP 4 699 459 A1**
(43) Date of publication of application: **25.02.2026**
(21) Application number: 25196588.5
(22) Date of filing: 19.08.2025
(51) Int. Cl.: A24D 3/06, A24D 3/10, D02G 1/12, D01F 2/00, D01F 2/24, D02G 3/44, D02G 3/48, D06M 15/05

(54) **LYOCELL MATERIAL, FILTER FOR SMOKING ARTICLES, SMOKING ARTICLE, AND MANUFACTURING METHODS THEREOF**

(30) Priority: 19.08.2024 KR 20240110605
(71) Applicant: Kolon Industries, Inc., Seoul 07793 (KR); KT&G Corporation, Daedeok-gu Daejeon 34337 (KR)
(72) Inventor: JEONG, Ji Eun, Seoul (KR); LEE, Jeong Hun, Seoul (KR); KWON, So Yeon, Seoul (KR); KIM, Seong Hun, Seoul (KR); JEONG, Jong Cheol, Seoul (KR); MA, Kyeng Bae, Daejeon (KR); KI, Sung Jong, Daejeon (KR); YANG, Jin Chul, Daejeon (KR); HA, Sung Hoon, Daejeon (KR); HWANG, Min Hee, Daejeon (KR)
(74) Representative: Isarpatent

(57) **Abstract**

The present application relates to a lyocell material, a filter for smoking articles, the filter including the lyocell material, and a smoking article including the filter. The lyocell material and the filter for smoking articles, according to the present application, may replace conventional cellulose acetate materials and filters for smoking articles including conventional cellulose acetate materials.

## Description

### Technical Field

The present application relates to a lyocell material, a filter including the same, a smoking article including the filter, and manufacturing methods thereof.

### Background Art

Until now, cellulose acetate fibers have been mainly used as cigarette filter materials. Cellulose acetate is known as a biodegradable material, but filters for smoking articles, which are made of cellulose acetate, remain in their original form for one to two years after being buried in soil, and it takes a considerable amount of time until they are completely biodegraded. Considering the amount and toxicity of tobacco products that are discarded and left in the living environment as well as tobacco products that are recovered as waste and landfilled after being used for smoking, it is necessary to further improve the biodegradability of filters for smoking articles. Accordingly, recently, a more environmentally friendly lyocell has been selected as a material to replace cellulose acetate.

### Disclosure of Invention

### Technical Problem

An object of the present application is to provide a lyocell material that can replace commercially available cellulose acetate for filters for smoking articles.

Another object of the present application is to provide a lyocell material for filters for smoking articles of which manufacturing process is environmentally friendly and which has excellent biodegradability upon disposal.

Another object of the present application is to provide a lyocell filter for smoking articles.

Another object of the present application is to provide a smoking article (for example, cigarette) including a lyocell filter.

### Solution to Problem

According to aspects of the present application, there may provide a lyocell material, a filter including the same, a smoking article, and the like.

According to an aspect of the present application, a lyocell material may be provided including a lyocell multifilament to which crimps are applied, the lyocell mateiral having a filtration index of 400 to 1000.

According to another aspect of the present application, a smoking article and/or a filter may be provided including a lyocell material having a filtration index of 400 to 1000.

According to another aspect of the present application, a smoking article may be provided including the lyocell material or the filter.

According to another aspect of the present application, methods of manufacturing the lyocell material, and the filter including the same, and the smoking article may be provided.

In this specification, 'smoking article' may refer to an article capable of generating aerosols, such as a cigarette, cigar, etc. In this regard, the smoking article may include an aerosol-generating material or an aerosol-forming substrate. Additionally, the smoking article may include a solid material based on a tobacco raw material, such as leaf tobacco, cut tobacco, reconstituted tobacco, etc. In addition, the smoking article may include a volatile compound.

Unless otherwise specifically defined in this specification, when the properties of a lyocell material, a filter for smoking articles, or components or compositions related thereto are affected by temperature, the temperature at which such properties are determined or measured may be room temperature. In this case, the room temperature is a temperature which is not particularly decreased or increased, for example, may be a temperature of 10 °C to 35 °C, particularly 15 °C to 35 °C, 20 °C to 30 °C, or about 25 °C.

As used herein, the term "crimp" or "crimped" may refer to the waviness, curliness, or undulating configuration imparted to materials such as fibers, (mono)filaments, multifilaments and/or yarns, inherently and/or through mechanical, thermal, or chemical processes. A crimp may be characterized by periodic deviations from a straight linear axis along the length of the material, fiber, (mono)filament, multifilament and/or yarn. One crimp of a material, fiber, (mono)filament, multifilament and/or yarn may be defined as one repetition unit of said periodic deviation. The presence of crimp contributes to properties such as elasticity, bulk, resilience, and texture in the material and fabrics made from it.

Hereinafter, the disclosure of the present application will be described in more detail.

The present application relates to a lyocell material. The lyocell material may be used in smoking articles, and, although not particularly limited, the lyocell material may be used in filters for smoking articles.

According to an aspect, there is provided a lyocell material including a lyocell multifilament to which crimps are applied, the lyocell material having a filtration index of 400 to 1000.

According to certain embodiments, a filtration index may be a value calculated according to Equation 1 below. $Filtration index = filling degree \times number of crimps$ in Equation 1,
the filling degree is a value obtained by dividing an actually measured weight of a lyocell material per unit volume by a theoretical weight of the lyocell material per unit volume and multiplying this value by one hundred.

According to certain embodiments, the filling degree in Equation 1 may be a value obtained by dividing an actually measured weight of the lyocell material per unit volume of a filter for smoking articles by a theoretical weight of the lyocell material per unit volume of the filter for smoking articles and multiplying this value by one hundred. In an exemplary lyocell material, the filling degree may be 15% to 30%.

According to certain embodiments, the filling degree may be 20% to 25%.

According to certain embodiments, the filling degree may be 21% to 24%.

According to certain embodiments, the filling degree may be 22% to 23%.

According to certain embodiments, the number of crimps may be 3.94 ea/cm (10 ea/inch) to 23.64 ea/cm (60 ea/inch).

According to certain embodiments, the number of crimps may be 9.84 ea/cm (25 ea/inch) to 23.64 ea/cm (60 ea/inch).

According to certain embodiments, the filling degree may be 15% to 30% and the number of crimps may be 5.91 ea/cm (15 ea/inch) to 23.64 ea/cm (60 ea/inch).

According to certain embodiments, the filling degree may be 21% to 24% and the number of crimps may be 7.87 ea/cm (20 ea/inch) to 17.72 ea/cm (45 ea/inch).

According to certain embodiments, the lyocell multifilament includes one or more monofilaments, and one or more of the monofilaments may have a non-circular cross-section.

According to certain embodiments, the lyocell multifilament includes one or more monofilaments, and all of the monofilaments may have a non-circular cross-section.

According to certain embodiments, the single fineness of the lyocell multifilament may be 1.67 dtex to 8.89 dtex (1.5 to 8.0 denier). The single fineness of a filament forming the lyocell multifilament refers to the monofilament fineness.

According to certain embodiments, the lyocell multifilament may have a total fineness of 1,667 tex to 6,111 tex (15,000 to 55,000 denier).

According to certain embodiments, the lyocell material may be a lyocell tow.

According to certain embodiments, the lyocell material may be used for a filter for smoking articles.

According to certain embodiments, the lyocell material may not be used for tire cords and/or clothes.

In addition, according to another aspect, there is provided a filter for smoking articles, the filter including any one of the lyocell materials as described in this application. In particular, the filtration index of the lyocell material included in the filter for smoking articles may be 400 to 1000.

Additionally, according to another aspect, there is provided a smoking article including any one of the filters for smoking articles as described in this application.

The lyocell material according to certain embodiment has a filtration index of 400 to 1000. By allowing the lyocell material to satisfy the above numerical range, the filter characteristics and processibility of a filter for smoking articles, the filter including the lyocell material, can be evenly improved.

In particular, by satisfying the above numerical range, the suction resistance and filter hardness of a filter for smoking articles, the filter including the lyocell material, may increase simultaneously. Furthermore, the process cost required for producing a filter including the lyocell material may be reduced. In particular, the time required for manufacturing a filter for smoking articles, the filter including the lyocell material, and the manufacturing cost per filter for smoking articles can be optimized and minimized.

Meanwhile, when the filtration index of the lyocell material is less than 400, the lyocell material may not provide sufficient suction resistance when included in a filter for smoking articles. In addition, the lyocell material may not provide sufficient filter hardness. As a result, a filter for smoking articles, the filter including lyocell material having a filtration index of less than 400, may not provide a high-quality user experience.

Conversely, when the filtration index of the lyocell material more than 1000, the cost required for manufacturing a filter for smoking articles, the filter including the lyocell material, may excessively increase. For example, the uniformity of the lyocell material may be impaired due to the excessive conditions in a crimp application process (crimping step), and as a result, the yield of the lyocell material to which crimps are applied may be decreased, and a post-processing process for stabilizing crimps may be additionally required. In addition, the filter paper of a filter for smoking articles, the filter including the lyocell material, may be burst due to the excessive compression and repulsion of the lyocell material, and the processability of filter manufacturing may be significantly reduced.

### [Non-circular cross-section]

At least one of the lyocell monofilaments included in the lyocell material of the present application may have a non-circular cross-section. The "non-circular" means that the shape of the outline of a cross-section is not circular, and the "cross-section" may be a cross-section obtained by cutting the lyocell monofilament virtually or actually perpendicular to the length direction of the filament.

The outline of the non-circular cross-section may come into contact with an imaginary first circle and an imaginary second circle, respectively. Additionally, the imaginary second circle may be within the imaginary first circle.

The imaginary first circle may be a circle having the smallest area value among the circles drawn to completely encompass one cross-section of a monofilament. The imaginary second circle may be a circle having the largest area value among the circles drawn within the cross section of the monofilament.

If a circumscribed circle including the cross section of the monofilament can be drawn, the imaginary first circle may be the above-described circumscribed circle. When an inscribed circle can be drawn within the cross section of the monofilament, the imaginary second circle may be the above-described inscribed circle.

The non-circular cross-section may have a shape including a plurality of protrusions, for example, a Y-shaped cross-section including three protrusions. It can be understood that the plurality of protrusions are formed integrally with the imaginary second circle as a center and that their ends are in contact with the imaginary first circle.

The non-circularity of a monofilament may be defined by Equation 1 below. $Non - circularity = r 1 / r 2$

Here, r1 is a radius of the imaginary first circle, and r2 is a radius of the imaginary second circle.

For example, the radius of the imaginary first circle may be 4 µm to 40 µm, the radius of the imaginary second circle may be 2 µm to 14 µm, and the non-circularity may be 1.01 to 10.

Additionally, the space occupancy of a monofilament may be defined by the following Equation 2. $Space occupancy = \left(S1/S2\right) \times 100 \left(%\right)$

Here, S1 is an area of the imaginary first circle, and S2 is a cross-sectional area of a monofilament included in a lyocell fiber.

For example, the space occupancy of a monofilament having a non-circular cross-section may be 120 % to 600 %.

### [Fineness]

The lyocell material of the present application includes a lyocell multifilament, and the lyocell multifilament may have a fineness suitable for manufacturing a filter for smoking articles and securing its function.

For example, the single fineness of a filament forming the lyocell multifilament may be 1.67 to 8.89 dtex (1.5 to 8.0 denier). In this case, the single fineness of the filament refers to a fineness of one monofilament separated from the lyocell multifilament. In other words, the single fineness of a filament forming the lyocell multifilament refers to the monofilament fineness.

Specifically, the single fineness of the filament may be, for example, 8.33 dtex (7.5 denier) or less, 7.78 dtex (7.0 denier) or less, 7.22 dtex (6.5 denier) or less, 6.67 dtex (6.0 denier) or less, 6.11 dtex (5.5 denier) or less, 5.56 dtex (5.0 denier) or less, 5.00 dtex (4.5 denier) or less, 3.89 dtex (3.5 denier) or less, 3.33 dtex (3.0 denier) or less, or 2.78 dtex (2.5 denier) or less. Further, the lower limit thereof may be, for example, 2.22 dtex (2.0 denier) or more, 2.78 dtex (2.5 denier) or more, 3.33 dtex (3.0 denier) or more, 3.89 dtex (3.5 denier) or more, 4.44 dtex (4.0 denier) or more, 5.00 dtex (4.5 denier) or more, 5.56 dtex (5.0 denier) or more, 6.11 dtex (5.5 denier) or more, 6.67 dtex (6.0 denier) or more, 7.22 dtex (6.5 denier) or more, or 7.78 dtex (7.0 denier) or more. Satisfying the above range may be more advantageous in securing stable physical properties (e.g., hardness or suction resistance implementation, etc.) and processability of a filter for smoking articles.

According to certain embodiments, the single fineness may be 2.22 to 8.33 dtex (2.0 denier to 7.5 denier), 2.78 to 8.33 dtex (2.5 denier to 7.5 denier), 3.33 to 8.33 dtex (3.0 denier to 7.5 denier), 3.89 to 8.33 dtex (3.5 denier to 7.5 denier), 4.44 to 8.33 dtex (4.0 denier to 7.5 denier), 5.00 to 8.33 dtex (4.5 denier to 7.5 denier), 5.56 to 8.33 dtex (5.0 denier to 7.5 denier), 6.11 to 8.33 dtex (5.5 denier to 7.5 denier), 6.67 to 8.33 dtex (6.0 denier to 7.5 denier), 7.22 to 8.33 dtex (6.5 denier to 7.5 denier), 7.78 to 8.33 dtex (7.0 denier to 7.5 denier), 2.22 to 7.78 dtex (2.0 denier to 7.0 denier), 2.78 to 7.78 dtex (2.5 denier to 7.0 denier), 3.33 to 7.78 dtex (3.0 denier to 7.0 denier), 3.89 to 7.78 dtex (3.5 denier to 7.0 denier), 4.44 to 7.78 dtex (4.0 denier to 7.0 denier), 5.00 to 7.78 dtex (4.5 denier to 7.0 denier), 5.56 to 7.78 dtex (5.0 denier to 7.0 denier), 6.11 to 7.78 dtex (5.5 denier to 7.0 denier), 6.67 to 7.78 dtex (6.0 denier to 7.0 denier), 7.22 to 7.78 dtex (6.5 denier to 7.0 denier), 2.22 to 7.22 dtex (2.0 denier to 6.5 denier), 2.78 to 7.22 dtex (2.5 denier to 6.5 denier), 3.33 to 7.22 dtex (3.0 denier to 6.5 denier), 3.89 to 7.22 dtex (3.5 denier to 6.5 denier), 4.44 to 7.22 dtex (4.0 denier to 6.5 denier), 5.00 to 7.22 dtex (4.5 denier to 6.5 denier), 5.56 to 7.22 dtex (5.0 denier to 6.5 denier), 6.11 to 7.22 dtex (5.5 denier to 6.5 denier), dtex (6.0 denier to 6.5 denier), 2.22 to 6.67 dtex (2.0 denier to 6.0 denier, 2.78 to 6.67 dtex (2.5 denier to 6.0 denier), 3.33 to 6.67 dtex (3.0 denier to 6.0 denier), 3.89 to 6.67 dtex (3.5 denier to 6.0 denier), 4.44 to 6.67 dtex (4.0 denier to 6.0 denier), 5.00 to 6.67 dtex (4.5 denier to 6.0 denier, 5.56 to 6.67 dtex (5.0 denier to 6.0 denier), 6.11 to 6.67 dtex (5.5 denier to 6.0 denier), 2.22 to 6.11 dtex (2.0 denier to 5.5 denier), 2.78 to 6.11 dtex (2.5 denier to 5.5 denier), 3.33 to 6.11 dtex (3.0 denier to 5.5 denier), 3.89 to 6.11 dtex (3.5 denier to 5.5 denier), 4.44 to 6.11 dtex (4.0 denier to 5.5 denier), 5.00 to 6.11 dtex (4.5 denier to 5.5 denier), 5.56 to 6.11 dtex (5.0 denier to 5.5 denier), 2.22 to 5.56 dtex (2.0 denier to 5.0 denier), 2.78 to 5.56 dtex (2.5 denier to 5.0 denier), 3.33 to 5.56 dtex (3.0 denier to 5.0 denier), 3.89 to 5.56 dtex (3.5 denier to 5.0 denier), 4.44 to 5.56 dtex (4.0 denier to 5.0 denier), 5.00 to 5.56 dtex (4.5 denier to 5.0 denier), 2.22 to 5.00 dtex (2.0 denier to 4.5 denier), 2.78 to 5.00 dtex (2.5 denier to 4.5 denier), 3.33 to 5.00 dtex (3.0 denier to 4.5 denier), 3.89 to 5.00 dtex (3.5 denier to 4.5 denier), 4.44 to 5.00 dtex (4.0 denier to 4.5 denier), 2.22 to 4.44 dtex (2.0 denier to 4.0 denier), 2.89 to 4.44 dtex (2.5 denier to 4.0 denier), 3.33 to 4.44 dtex (3.0 denier to 4.0 denier), 3.89 to 4.44 dtex (3.5 denier to 4.0 denier), 2.22 to 3.89 dtex (2.0 denier to 3.5 denier), 2.78 to 3.89 dtex (2.5 denier to 3.5 denier), 3.33 to 3.89 dtex (3.0 denier to 3.5 denier), 2.22 to 3.33 dtex (2.0 denier to 3.0 denier), 2.78 to 3.33 dtex (2.5 denier to 3.0 denier), or 2.22 to 2.78 dtex (2.0 denier to 2.5 denier).

According to certain embodiments, the total fineness of the lyocell material may be 1,667 to 6,111 tex (15,000 to 55,000 denier), and the total fineness of the lyocell material may be calculated as the sum of the finenesses of the lyocell monofilaments. For example, the lower limit of the total fineness may be, for example, 1,778 tex (16,000 denier) or more, 1,833 tex (16,500 denier) or more, 1,889 tex (17,000 denier) or more, 1,944 tex (17,500 denier) or more, 2,000 tex (18,000 denier) or more, 2,056 tex (18,500 denier) or more, 2,111 tex (19,000 denier) or more, 2,167 tex (19,500 denier) or more, 2,222 tex (20,000 denier) or more, 2,278 tex (20,500 denier) or more, 2,333 tex (21,000 denier) or more, 2,389 tex(21,500 denier) or more, 2,444 tex(22,000 denier) or more, 2,500 tex(22,500 denier) or more, 2,556 tex(23,000 denier) or more, 2,611 tex(23,500 denier) or more, 2,667 tex(24,000 denier) or more, 2,722 tex(24,500 denier) or more, 2,778 tex(25,000 denier) or more, 2,833 tex(25,500 denier) or more, 2,889 tex(26,000 denier) or more, 2,944 tex(26,500 denier) or more, 3,000 tex(27,000 denier) or more, 3,056 tex(27,500 denier) or more, 3,111 tex(28,000 denier) or more, 3,167 tex(28,500 denier) or more, 3,222 tex(29,000 denier) or more, 3,287 tex(29,500 denier) or more, 3,333 tex(30,000 denier) or more, 3,389 tex(30,500 denier) or more, 3,444 tex(31,000 denier) or more, 3,500 tex(31,500 denier) or more, 3,556 tex(32,000 denier) or more, 3,611 tex(32,500 denier) or more, 3,667 tex(33,000 denier) or more, 3,722 tex(33,500 denier) or more, 3,778 tex(34,000 denier) or more, 3,833 tex(34,500 denier) or more, 3,889 tex(35,000 denier) or more, 3,944 tex(35,500 denier) or more, 4,000 tex(36,000 denier) or more, 4,056 tex(36,500 denier) or more, 4,111 tex(37,000 denier) or more, 4,167 tex(37,500 denier) or more, 4,222 tex(38,000 denier) or more, 4,278 tex(38,500 denier) or more, 4,333 tex(39,000 denier) or more, 4,389 tex(39,500 denier) or more, 4,444 tex(40,000 denier) or more, 4,500 tex(40,500 denier) or more, 4,556 tex(41,000 denier) or more, 4,611 tex(41,500 denier) or more, 4,667 tex(42,000 denier) or more, 4,722 tex(42,500 denier) or more, 4,778 tex(43,000 denier) or more, 4,833 tex(43,500 denier) or more, 4,889 tex(44,000 denier) or more, 4,944 tex(44,500 denier) or more, 5,000 tex(45,000 denier) or more, 5,056 tex(45,500 denier) or more, 5,111 tex(46,000 denier) or more, 5,167 tex(46,500 denier) or more, 5,222 tex(47,000 denier) or more, 5,278 tex(47,500 denier) or more, 5,333 tex(48,000 denier) or more, 5,389 tex(48,500 denier) or more, 5,444 tex(49,000 denier) or more, 5,500 tex(49,500 denier) or more, 5,556 tex(50,000 denier) or more, 5,611 tex(50,500 denier) or more, 5,667 tex(51,000 denier) or more, 5,722 51,500 denier or more, 5,778 tex (52,000 denier) or more, 5,833 tex (52,500 denier) or more, 5,889 tex (53,000 denier) or more, 5,944 tex (53,500 denier) or more, 6,000 tex (54,000 denier) or more, or 6,056 tex (54,500 denier) or more. Further, the upper limit thereof may be, for example, 6,056 tex (54,500 denier) or less, 6,000 tex (54,000 denier) or less, 5,944 tex (53,500 denier) or less, 5,889 tex (53,000 denier) or less, 5,833 tex (52,500 denier) or less, 5,778 tex (52,000 denier) or less, 5,722 tex (51,500 denier) or less, 5,667 tex (51,000 denier) or less, 5,611 tex (50,500 denier) or less, 5,556 tex (50,000 denier) or less, 5,500 tex (49,500 denier) or less, 5,444 tex(49,000 denier) or less, 5,389 tex(48,500 denier) or less, 5,333 tex(48,000 denier) or less, 5,278 tex(47,500 denier) or less, 5,222 tex(47,000 denier) or less, 5,167 tex(46,500 denier) or less, 5,111 tex(46,000 denier) or less, 5,056 tex(45,500 denier) or less, 5,000 tex(45,000 denier) or less, 4,944 tex(44,500 denier) or less, 4,889 tex(44,000 denier) or less, 4,833 tex(43,500 denier) or less, 4,778 tex (43,000 denier) or less, 4,722 tex (42,500 denier) or less, 4,667 tex (42,000 denier) or less, 4,611 tex (41,500 denier) or less, 4,556 tex (41,000 denier) or less, 4,500 tex (40,500 denier) or less, 4,444 tex (40,000 denier) or less, 4,389 tex (39,500 denier) or less, 4,333 tex (39,000 denier) or less, 4,278 tex (38,500 denier) or less, 4,222 tex (38,000 denier) or less, 4,167 tex (37,500 denier) or less, 4,111 tex (37,000 denier) or less, 4,056 tex (36,500 denier) or less, 4,000 tex (36,000 denier) or less, 3,944 tex (35,500 denier) or less, 3,889 tex (35,000 denier) or less, 3,833 tex (34,500 denier) or less, 3,778 tex (34,000 denier) or less, 3,722 tex (33,500 denier) or less, 3,667 tex (33,000 denier) or less, 3,611 tex (32,500 denier) or less, 3,556 tex (32,000 denier) or less, 3,500 tex (31,500 denier) or less, 3,444 tex (31,000 denier) or less, 3,389 tex (30,500 denier) or less, 3,333 tex (30,000 denier) or less, 3,278 tex (29,500 denier) or less, 3,222 tex (29,000 denier) or less, 3,167 tex (28,500 denier) or less, 3,111 tex (28,000 denier) or less, 3,056 tex (27,500 denier) or less, 3,000 tex (27,000 denier) or less, 2,944 tex (26,500 denier) or less, 2,889 tex (26,000 denier) or less, 2,833 tex (25,500 denier) or less, 2,778 tex (25,000 denier) or less, 2,722 tex (24,500 denier) or less, 2,667 tex (24,000 denier) or less, 2,611 tex (23,500 denier) or less, 2,556 tex (23,000 denier) or less, 2,500 tex (22,500 denier) or less, 2,444 tex (22,000 denier) or less, 2,389 tex (21,500 denier) or less, 2,333 tex (21,000 denier) or less, 2,278 tex (20,500 denier) or less, 2,222 tex (20,000 denier) or less, 2,167 tex (19,500 denier) or less, 2,111 tex (19,000 denier) or less, 2,056 tex (18,500 denier) or less, 2,000 tex (18,000 denier) or less, 1,944 tex (17,500 denier) or less, 1,889 tex (17,000 denier) or less, 1,833 tex (16,500 denier) or less, 1,778 tex (16,000 denier) or less, or 1,722 tex (15,500 denier) or less. When the total fineness is outside the above range, the processability of manufacturing a filter for smoking articles may not be good (continuous process by cutting is impossible), and when the amount of tow filling a filter wrapping paper during a process of manufacturing a filter for smoking articles may be too small or too large, it may be difficult to secure sufficient properties (e.g., hardness or suction resistance, etc.) of the filter.

Although there are no particular restrictions on the method of measuring fineness, for example, a 2 m sample is collected from the lyocell material to be measured, for example, a lyocell tow, and is left and stabilized in a room with a temperature condition of 20±2°C and a humidity condition of 65±4%RH for 24 hours. One end of the stabilized lyocell tow is fixed, and the other end thereof is provided with a 2 kg of weight. After the tow is maintained and stabilized for 5 seconds in an extended state due to a load, it is cut into 90 cm pieces to obtain a sample, and the weight of the sample (total fineness) is measured. According to a denier conversion method, the total fineness is calculated by multiplying the measured weight by 10,000. When the total fineness of the sample is divided by the number of monofilaments in the same, the single fineness of a monofilament in the sample is calculated.

As described above, the total fineness of the lyocell multifilament may be determined by the single fineness of the monofilament and the number of crimps. In the present application, the single fineness and the number of crimps may be controlled, and the total fineness of the tow suitable for manufacturing a filter for smoking articles and securing its function may be secured.

### [Number of crimps]

According to certain embodiments, the lyocell multifilament may have crimps of 3.94 to 23.62 per centimeter (10 to 60 per inch). The unit "ea/inch (ea/cm)" refers to the number of crimps per unit length (inch or rather cm), wherein the term "ea" refers to the number of crimps. For example, the number of crimps may be 5.91 ea/cm(15 ea/inch) or more, 7.87 ea/cm(20 ea/inch) or more, 9.84 ea/cm(25 ea/inch) or more, 11.81 ea/cm(30 ea/inch) or more, 13.78 ea/cm(35 ea/inch) or more, 15.75 ea/cm(40 ea/inch) or more, or 17.72 ea/cm(45 ea/inch) or more, and the upper limit thereof may be, for example, 21.69 ea/cm(55 ea/inch) or less, 19.69 ea/cm(50 ea/inch) or less, 17.72 ea/cm(45 ea/inch) or less, 15.75 ea/cm(40 ea/inch) or less, 13.78 ea/cm(35 ea/inch) or less, 11.81 ea/cm(30 ea/inch) or less, or 9.84 ea/cm(25 ea/inch) or less. The number of crimps and the uniformity thereof may be controlled through pressure and temperature conditions, etc., in the crimping process to be described below.

Although not particularly limited, the number of crimps may be measured using, for example, a single fiber property evaluation apparatus (for example, Favimat). Specifically, the manufactured lyocell material (preferably lyocell tow) sample may be left and stabilized for 24 hours under conditions of a temperature of 20±2°C and a humidity of 65±4%. A specimen may be collected from the stabilized sample without damaging the crimps. The collected specimen may be mounted on a dedicated jig with a length (gauge length) of 10 to 30 mm. At measurement, the initial load may be 0.45 g/tex (0.05 g/denier), and the crimp sensitivity at measurement may be 0.01 mm. The number of crimps may be measured under the above-described conditions (that is, temperature of 20±2°C, humidity of 65±4%).

Although not particularly limited, the lyocell material manufactured to satisfy the single fineness, total fineness, and/or the number of crimps, described above, may be used in smoking articles.

### [Lyocell material]

According to certain embodiments, there is provided a lyocell material including a lyocell multifilament to which crimps are applied, the lyocell material having a filtration index of 400 to 1000. By allowing the lyocell material to satisfy the above-described numerical range, the filter characteristics and processibility of a filter for smoking articles, the filter including the lyocell material, can be evenly improved.

According to certain embodiments, the lower limit of the filtration index may be 260 or more, 270 or more, 280 or more, 290 or more, 300 or more, 310 or more, 320 or more, 330 or more, 340 or more, 350 or more, 360 or more, 370 or more, 380 or more, 390 or more, 400 or more, 410 or more, 420 or more, 430 or more, 440 or more, 450 or more, 460 or more, 470 or more, 480 or more, 490 or more, 500 or more, 510 or more, 520 or more, 530 or more, 540 or more, or 550 or more. The upper limit of the filtration index may be 590 or less, 580 or less, 570 or less, 560 or less, 550 or less, 540 or less, 530 or less, 520 or less, 510 or less, 500 or less, 490 or less, 480 or less, 470 or less, 460 or less, 450 or less, 440 or less, 430 or less, 420 or less, 410 or less, 400 or less, 390 or less, 380 or less, 370 or less, 360 or less, 350 or less, 340 or less, 330 or less, 320 or less, 310 or less, or 300 or less.

Meanwhile, when the filtration index of the lyocell material is less than 300, the lyocell material may not provide sufficient filter characteristic (e.g., suction resistance, filter hardness, etc.) when included in a filter for smoking articles. Conversely, when the filtration index of the lyocell material more than 600, the cost (e.g., yield, process time, etc.) required for manufacturing a filter for smoking articles, the filter including the lyocell material, may excessively increase.

According to certain embodiments, the filtration index may be a value calculated according to Equation 1 below. $Filtration index = filling degree \times number of crimps$

in Equation 1,
the filling degree is a value obtained by dividing an actually measured weight of a lyocell material per unit volume by a theoretical weight of the lyocell material per unit volume and multiplying this value by one hundred. More preferably, the filling degree in Equation 1 may be a value obtained by dividing an actually measured weight of the lyocell material per unit volume of a filter for smoking articles by a theoretical weight of the lyocell material per unit volume of the filter for smoking articles and multiplying this value by one hundred.

In particular, since the filling degree in Equation 1 may be calculated by dividing an actually measured weight of the lyocell material per unit volume of a filter for smoking articles by a theoretical weight of the lyocell material per unit volume of the filter for smoking articles and multiplying this value by one hundred, the relative content of the lyocell material included in the filter for smoking articles may be evaluated based on the theoretical value and the actually measured value.

The theoretical weight of the lyocell material per unit volume can be calculated using the density of the lyocell material and the volume of a lyocell material used for preparing a filter for smoking articles, wherein the density of the lycell material can be 0.7 to 0.8 g/cm³, preferably 0.749 g/cm³.

The actually measured weight can be determined by weighing the lyocell material actually used to prepare a filter for smoking articles.

According to certain embodiments, the filling degree may be 15% to 30%. For example, the lower limit of the filling degree may be 16% or more, 17% or more, 18% or more, 19% or more, 20% or more, 21% or more, or 22% or more, and the upper limit of the filling degree may be 29% or less, 28% or less, 27% or less, 26% or less, 25% or less, 24% or less, or 23% or less.

By including the lyocell material in a filter for smoking articles such that the filling degree satisfies the above range, the filter hardness of the filter for smoking articles can be implemented at a certain level or higher, and a high-quality feeling of use can be provided to the user.

Meanwhile, when the filling degree is less than 15%, the hardness and suction resistance of the filter for smoking articles may decrease due to a lack of the lyocell material, and thus the usability of the user may deteriorate. Conversely, when the filling degree more than 30%, the filter paper of the filter for smoking articles may burst due to the excessive amount of the lyocell material, and a process cost may increase.

According to certain embodiments, the number of crimps may be 3.94 ea/cm to 23.62 ea/cm (10 ea/inch to 60 ea/inch), preferably, the number of crimps may be 9.84 ea/cm to 19.69 ea/cm (25 ea/inch to 50 ea/inch), and more preferably, the number of crimps may be 13.78 ea/cm to 17.72 ea/cm (35 ea/inch to 45 ea/inch).

As the number of crimps increases, the filling degree may decrease. However, when the number of crimps exceeds 23.62 ea/cm (60 ea/inch), a harsh crimp application process may be required to provide excessive crimps. As a result, a process cost may increase due to the crimp application process, and the yield of the lyocell material to which crimps are applied may decrease.

According to a preferred embodiment, a lyocell material has a filling degree of 15% to 30% and a crimp number of 5.91 ea/cm to 23.62 ea/cm (15 ea/inch to 60 ea/inch). Further, according to another preferred embodiment, a lyocell material has a filling degree of 21% to 24% and a crimp number of 7.87 ea/cm to 17.72 ea/cm (20 ea/inch to 45 ea/inch). By having the filling degree and the number of crimps satisfying the above ranges, the filter characteristics of a filter for smoking articles, the filter including the lyocell material, can be improved, and a reduction in the process cost for producing the same can be achieved at the same time.

Meanwhile, the lyocell material as described in the application may be used for purposes other than tire cords and/or clothes by satisfying a given filtration index. Referring to the definition of filtration index, it is not possible to determine whether lyocell material for tire cords or the lyocell material for clothes satisfies the filtration index. In addition, it is obvious that the definition of filtration index cannot be derived from the lyocell material for tire cords or the lyocell material for clothes.

### [Binder]

According to certain embodiments, the lyocell material may further include a binder. The binder may be present, for example, on the surface of the lyocell multifilament, or between the lyocell multifilaments (or between monofilaments). The binder may increase the hardness of a filter for smoking articles, thereby preventing a filter from being caught during a process of manufacturing a filter or a process of manufacturing a smoking article (for example, cigarette).

The type of a usable binder is not particularly limited, and any known binder may be used as long as it does not hinder the purpose of the present invention. For example, a binder providing sufficient compatibility with an oil used in the present application, improving the hardness of a filter, and providing excellent binding force may be used.

According to certain embodiments, the binder may include a polyester-based binder, a cellulosic-based binder, and/or a vinyl-based binder.

According to certain embodiments, a polyester-based binder including at least one selected from the group consisting of alkylene, arylene and heteroarylene, each having 5 to 12 carbon atoms, may be used.

Examples of the cellulose-based binder may include, but are not limited to, hydroxypropyl methyl cellulose (HPMC), ethyl cellulose (EC), methyl cellulose (MC), and/or carboxymethyl cellulose (CMC). According to certain embodiments, the cellulose-based binder is selected from the group consisting of hydroxypropyl methyl cellulose (HPMC), ethyl cellulose (EC), methyl cellulose (MC), carboxymethyl cellulose (CMC), or a combination thereof.

Examples of the vinyl-based binder may include, but are not limited to, polyvinylpyrrolidone (PVP), polyvinyl alcohol (PVA), and/or ethylene vinyl acetate (EVAc).

A method of applying (coating) the binder to a lyocell material will be described later. According to certain embodiments, the vinyl-based binder is selected from the group consisting of polyvinylpyrrolidone (PVP), polyvinyl alcohol (PVA), ethylene vinyl acetate (EVAc), or a combination thereof.

### [Oil]

According to certain embodiments, the lyocell material may include a lyocell multifilament; and an oil applied onto the lyocell multifilament. The oil includes (a) an esterification product of a fatty acid having 16 or more carbon atoms and an aliphatic monohydric alcohol; and (b) an esterification product of sorbitan and a fatty acid having 16 or more carbon atoms. This oil may be applied to some or all of monofilaments or multifilaments constituting the lyocell material. Additionally, the oil may penetrate among filaments.

The oil including at least the component (a) and the component (b) may have hydrophobicity. As a result, the lyocell material treated with the oil has excellent spreading properties.

In an embodiment of the present application, the lyocell material may include a preset content of the oil. In this case, the content of the oil may refer to OPU (wt%) to be described later. "OPU" may refer to "oil pick up ratio". According to certain embodiments, the lyocell material may include an oil in a content of 0.1 wt% or more based on 100 wt% of the total lyocell material. For example, the content of the oil may be 0.5 wt% or more, 1.0 wt% or more, 1.5 wt% or more, 2.0 wt% or more, 2.5 wt% or more, 3.0 wt% or more, specifically, 3.5 wt% or more, 4.0 wt% or more, 4.2 wt% or more, 4.5 wt% or more, 5.0 wt% or more, 5.5 wt% or more, 6.0 wt% or more, 6.5 wt% or more, 7.0 wt% or more, 7.5 wt% or more, 8.0 wt% or more, 8.5 wt% or more, 9.0 wt% or more, or 9.5 wt% or more. Further, the upper limit thereof may be, for example, 20.0 wt% or less, 18.0 wt% or less, 17.0 wt% or less, 16.0 wt% or less, 15.0 wt% or less, 14.5 wt% or less, 14.0 wt% or less, 13.5 wt% or less, 13.0 wt% or less, 12.5 wt% or less, 12.0 wt% or less, 11.5 wt% or less, 11.0 wt% or less, 10.5 wt% or less, 10 wt% or less, 9.5 wt% or less, 9.0 wt% or less, 8.5 wt% or less, 8.0 wt% or less, 7.8 wt% or less, or 7.6 wt% or less.

As a method of measuring the content (OPU) of the oil, for example, an extrusion method may be used. For example, a sample (e.g., 2 to 5 g, specifically about 2.5 g) is collected (in this case, the weight of the collected sample is referred to as a sample weight), and is introduced into a syringe-shaped container. The material of the container is not particularly limited, but may be SUS (stainless steel). Subsequently, a solvent (e.g., methanol) is introduce into the container containing the sample (the amount of the introduced solvent may be 10 ml or less (e.g., about 8 ml)). When adding the solvent to the sample, a dropping method may be used, and a dropping speed may be adjusted uniformly. And, as described above, the solvent introduced into the container is allowed to drop from one end of the syringe-shaped container onto a plate. In this case, the plate is pre-weighed (the weighed weight is referred to as plate weight A), and the plate is mounted so that the solvent dropped onto the plate can fly away (i.e., evaporate) at a temperature of 120°C to 130°C (e.g., 125°C). The introduction and dropping of the solvent are performed three times, and the sample is pressed once using a syringe-shaped container to apply pressure (e.g., 98 N/cm² (10 kgf/cm²) or less, 49 N/cm² (5 kgf/cm²) or less, or 20-39 N/cm² (2-4 kgf/cm²)) to the sample. This process allows the solvent and oil present in the sample to be sufficiently extruded. The sample is squeezed under pressure until no solvent comes out. Then, the plate is stored in a desiccator for 5 to 10 minutes, and the weight of the plate containing the sample (plate weight B) is measured. Then, the content of the oil is calculated according to Equation below. $\begin{matrix}Content of oil by extrusion \left(OPU, % or wt%\right) \\ = \left\{\left(plate weight B-plate weight A\right)/\left(sample weight\right)\right\} \times 100\end{matrix}$

In addition, the lyocell material that serves as the standard for the content of the oil may be at least an oil-treated lyocell multifilament. For example, the lyocell material may be a lyocell multifilament to which a first oil treatment (as described below) has been applied, a lyocell multifilament to which a first oil treatment and a second oil treatment (as described below) have been applied, or a lyocell multifilament to which a binder treatment to be described below has been applied together with the above-described oil treatment. Additionally, the lyocell multifilament treated with an oil and/or a binder may be a lyocell multifilament to which crimps are applied.

In relation to the oil of the present application, the component (a) may be a compound that can function as a type of lubricant or oil, and may be a component that may be harmless to the human body enough to be used in food. The component (a) provides lubricity to fibers introduced into a crimper. When lubricity is insufficient, lyocells may clump together and not pass through the crimper, and when lubricity is too high, crimps may not form properly. Taking these functions into consideration, the content of the component (a) may be controlled as described below.

In relation to the component (a), the type of fatty acid having 16 or more carbon atoms forming the esterification product is not particularly limited. Fatty acids having 16 or more carbon atoms may be used as long as they provide esterification products that may be harmless to the human body to such a degree of being used in foods.

For example, as the fatty acids having 16 or more carbon atoms, saturated fatty acids and/or unsaturated fatty acids may be used.

Examples of saturated fatty acids may include palmitic acid (hexadecanoic acid, CH₃(CH₂)₁₄COOH), margaric acid (heptadecanoic acid, CH₃(CH₂)₁₅COOH), stearic acid (octadecanoic acid, CH₃(CH₂)₁₆COOH), nonadecylic acid (nonadecanoic acid, CH₃(CH₂)₁₇COOH), and arachidic acid (eicosanoic acid, CH₃(CH₂)₁₈COOH). However, the types of available saturated fatty acids are not limited thereto. According to certain embodiments the saturated fatty acid is selected from the group consisting of palmitic acid (hexadecanoic acid, CH₃(CH₂)₁₄COOH), margaric acid (heptadecanoic acid, CH₃(CH₂)₁₅COOH), stearic acid (octadecanoic acid, CH₃(CH₂)₁₆COOH), nonadecylic acid (nonadecanoic acid, CH₃(CH₂)₁₇COOH), arachidic acid (eicosanoic acid, CH₃(CH₂)₁₈COOH), or a combination thereof.

Examples of unsaturated fatty acids may include palmitoleic acid (CH₃(CH₂)₅CH=CH(CH₂)₇COOH), oleic acid (CH₃(CH₂)₇CH=CH(CH₂)₇COOH), linoleic acid (C₁₈H₃₂O₂), and arachidonic acid (C₂₀H₃₂O₂). However, the types of available unsaturated fatty acids are not limited thereto.

According to certain embodiments the unsaturated fatty acid is selected from the group consisting of palmitoleic acid (CH₃(CH₂)₅CH=CH(CH₂)₇COOH), oleic acid (CH₃(CH₂)₇CH=CH(CH₂)₇COOH), linoleic acid (C₁₈H₃₂O₂), arachidonic acid (C₂₀H₃₂O₂), or combination thereof.

In some embodiments, the fatty acid is selected from the group consisting of palmitic acid, margaric acid, stearic acid, nonadecylic acid, arachidic acid, palmitoleic acid, oleic acid, linoleic acid, and arachidonic acid.

According to certain embodiments, the upper limit of the number of carbons of the fatty acid having 16 or more carbon atoms is not particularly limited, but may be, for example, 40 or less, 36 or less, 32 or less, 28 or less, 24 or less, or 20 or less.

In relation to the component (a), the type of aliphatic monohydric alcohol forming it is also not particularly limited. Aliphatic monohydric alcohols capable of providing esterification products that are harmless to the human body to such a degree of being used in foods may be used.

In some embodiments, saturated fatty alcohols or unsaturated fatty alcohols may be used, and they may have a linear or branched form.

According to certain embodiments, the number of carbon atoms of the aliphatic monohydric alcohol may be 1 to 40. Specifically, the number of carbon atoms of the aliphatic monohydric alcohol may be, for example, 4 or more, 8 or more, 12 or more, 16 or more, or 20 or more.

Examples of the aliphatic monohydric alcohols may include, but are not limited to, methanol, ethanol, butanol, lauryl alcohol, isotridecanol, and stearyl alcohol. In some embodiments, the aliphatic monohydric alcohol is selected from the group consisting of methanol, ethanol, butanol, lauryl alcohol, isotridecanol, and stearyl alcohol.

In some embodiments of the present application, as the component (a), an esterification product of isotridecanol and stearic acid (e.g., isotridecyl stearate) may be used. However, the types of available component (a) are not limited thereto.

As will be described below, the content of the component (a) included in the oil may be adjusted in consideration of the function of the oil or the function of the component (a).

The component (b), i.e., an ester of sorbitan and fatty acid having 16 or more carbon atoms, can be a compound that can function as a type of emulsifier, and may be a component that may be harmless to the human body to such a degree of being used in foods.

Since this component (b) has both hydrophilicity and hydrophobicity due to polyhydric alcohol (i.e., sorbitan), it enables the component (a) providing lubricity to fibers to be well dispersed in water to be described below. In addition, the components (a) and (b) used together not only increase the dispersibility of the oil as described above, but also lower the melting point of the oil, thereby ensuring the handling easiness and stability of the oil. Taking these functions into consideration, the content of the component (b) may be controlled as will be described below.

In relation to the component (b), the type of fatty acid having 16 or more carbon atoms forming it is not particularly limited. Fatty acids having 16 or more carbon atoms capable of providing esterification products that may be harmless to the human body to such a degree of being used in foods may be used.

According to certain embodiments, as the fatty acids having 16 or more carbon atoms, saturated fatty acids and/or unsaturated fatty acids may be used.

Examples of saturated fatty acids may include palmitic acid (hexadecanoic acid, CH₃(CH₂)₁₄COOH), margaric acid (heptadecanoic acid, CH₃(CH₂)₁₅COOH), stearic acid (octadecanoic acid, CH₃(CH₂)₁₆COOH), nonadecylic acid (nonadecanoic acid, CH₃(CH₂)₁₇COOH), and arachidic acid (eicosanoic acid, CH₃(CH₂)₁₈COOH). According to certain embodiments, the saturated fatty acid is selected from the group consisting of palmitic acid (hexadecanoic acid, CH₃(CH₂)₁₄COOH), margaric acid (heptadecanoic acid, CH₃(CH₂)₁₅COOH), stearic acid (octadecanoic acid, CH₃(CH₂)₁₆COOH), nonadecylic acid (nonadecanoic acid, CH₃(CH₂)₁₇COOH), arachidic acid (eicosanoic acid, CH₃(CH₂)₁₈COOH), or a combination thereof. However, the types of available saturated fatty acids are not limited thereto.

Examples of unsaturated fatty acids may include palmitoleic acid (CH₃(CH₂)₅CH=CH(CH₂)₇COOH), oleic acid (CH₃(CH₂)₇CH=CH(CH₂)₇COOH), linoleic acid (C₁₈H₃₂O₂), and arachidonic acid (C₂₀H₃₂O₂). In certain embodiments, the unsaturated fatty acid is selected from the group consisting of palmitoleic acid (CH₃(CH₂)₅CH=CH(CH₂)₇COOH), oleic acid (CH₃(CH₂)₇CH=CH(CH₂)₇COOH), linoleic acid (C₁₃H₃₂O₂), arachidonic acid (C₂₀H₃₂O₂), or a combination thereof. However, the types of available unsaturated fatty acids are not limited thereto. In some embodiments, the fatty acid is selected from the group consisting of palmitic acid, margaric acid, stearic acid, nonadecylic acid, arachidic acid, palmitoleic acid, oleic acid, linoleic acid, and arachidonic acid.

The upper limit of the number of carbons of the fatty acid having 16 or more carbon atoms is not particularly limited, but may be, for example, 40 or less, 36 or less, 32 or less, 28 or less, 24 or less, or 20 or less.

According to some embodiments, as the component (b), an esterification product of sorbitan and oleic acid (e.g., sorbitan monooleate) may be used. However, the type of the available component (b) is not limited thereto.

The content of the component (b) may be adjusted in consideration of the function of the component (b) and the function of the oil as described above.

In some embodiments, the oil may include 20 to 60 parts by weight of an ester esterification product (b) of sorbitan and a fatty acid having 16 or more carbon atoms with respect to 100 parts by weight of an esterification product (a) of a fatty acid having 16 or more carbon atoms and an aliphatic monohydric alcohol.

For example, the oil of the present application may include the component (b) in a content of 25 parts by weight or more, 30 parts by weight or more, 35 parts by weight or more, 40 parts by weight or more, 45 parts by weight or more, or 50 parts by weight or more with respect to 100 parts by weight of the component (a). Further, the upper limit of the content of the component (b) with respect to 100 parts by weight of the component (a) may be, for example, 55 parts by weight or less, 50 parts by weight or less, 45 parts by weight or less, 40 parts by weight or less, 35 parts by weight or less, 30 parts by weight or less, or 25 parts by weight or less. When the above content range is satisfied, the surface of the lyocell multifilament or lyocell tow treated with the oil may have hydrophobicity.

For example, the oil may include 40 to 80 wt% of an esterification product (a) of a fatty acid having 16 or more carbon atoms and an aliphatic monohydric alcohol, based on 100 wt% of the total weight of the oil. For example, the content of the component (a) may be 45 wt% or more, 50 wt% or more, 55 wt% or more, 60 wt% or more, or 65 wt% or more, 70 wt% or more, or 75 wt% or more, based on 100 wt% of the total weight of the oil. Further, the upper limit of the content thereof may be, for example, 75 wt% or less, 70 wt% or less, 65 wt% or less, 60 wt% or less, 55 wt% or less, 50 wt% or less, or 45 wt% or less.

In some embodiments, the oil may include an excess amount of the component (a).

In some embodiments, the oil may include 15 to 55 wt% of an esterification product (b) of sorbitan and a fatty acid having 16 or more carbon atoms, based on 100 wt% of the total weight of the oil. For example, the content of the component (b) may be 20 wt% or more, 25 wt% or more, 30 wt% or more, 35 wt% or more, 40 wt% or more, 45 wt% or more, or 50 wt% or more, based on 100 wt% of the total weight of the oil. Further, the upper limit of the content thereof may be, for example, 50 wt% or less, 45 wt% or less, 40 wt% or less, 35 wt% or less, 30 wt% or less, or 25 wt% or less.

In some embodiments, the oil may further include water. A small amount of water may help emulsification.

The content of water is not particularly limited, but water may be included in the amount remaining after excluding the total content of components (a) and (b) from 100 wt% of the entire oil. The content of water in the oil (i.e., the remaining amount excluding the total content of the remaining components excluding water) may be, for example, 10 wt% or less, 9 wt% or less, 8 wt% or less, 7 wt% or less, 6 wt% or less, 5 wt% or less, 4 wt% or less, 3 wt% or less, 2 wt% or less, or 1 wt% or less. Further, the lower limit thereof may be, for example, 0 wt% or more, 0.1 wt% or more, 0.5 wt% or more, or 1 wt% or more.

### [Method of manufacturing lyocell material]

This application relates to a method of manufacturing a lyocell material. By this method, a lyocell material may be manufactured, and this lyocell material may be used in smoking articles.

According to certain embodiments, the method of manufacturing a lyocell material includes a step of spinning lyocell dope; a step of coagulating and obtaining multifilament; a step of washing; a step of oil treatment; and step of applying a crimp (crimping step). The step of apply a crimp can be referred to a step of imparting a crimp. Further, the method of manufacturing a lyocell material may further include a step of binder treatment; and one or more other steps.

The oil treatment step may be performed before the crimp application step, after the crimp application step, or before and after the crimp application step.

The oil treatment may be performed independently, for example, by spraying an oil of the above-described composition onto lyocell multifilaments or by immersing the lyocell multifilaments in the oil. The oil treatment may be performed so that the content (e.g., OPU (wt%)) of the oil in the lyocell material satisfies a preset range, as described above.

The crimp application step may be performed, for example, by applying steam and/or pressure to the lyocell multifilaments.

A method of manufacturing a lyocell material according to a certain embodiments of the present application, including an oil treatment step and a crimp application step, will be described in more detail below. The method of the present application may be performed by including one or more of the steps to be described below.

### <(a) Lyocell dope spinning step>

This step is a step of spinning a lyocell spinning dope including lyocell cellulose (or cellulose pulp) and N-methylmorpholine-N-oxide (NMMO).

Commercially available cellulose acetate filters are pointed out as a major cause of microplastics. However, just as an amine oxide solvent used in the production of lyocell fibers is recyclable and is biodegradable even when it is discarded, a lyocell material does not generate any pollutants during its production process. Furthermore, since a lyocell tow is biodegraded within a relatively short period of time and is removed, lyocell is a more environmentally friendly material than cellulose acetate.

According to certain embodiments, the content of cellulose in the spinning dope may be 5 to 15 wt% based on 100 wt% of the total weight of the lyocell dope. When the content of cellulose is too small, it is difficult to implement the characteristics of lyocell fibers, and when the content of cellulose exceeds the above range, it is difficult to dissolve in a solvent. Considering this, the content of cellulose in the spinning dope may be, for example, 6 wt% or more, 7 wt% or more, 8 wt% or more, 9 wt% or more, or 10 wt% or more, based on 100 wt% of the total weight of the lyocell dope, and the upper limit thereof may be, for example, 14 wt% or less, 13 wt% or less, 12 wt% or less, 11 wt% or less, 10 wt% or less, or 9 wt% or less, based on 100 wt% of the total weight of the lyocell dope. The term "cellulose" may refer to "lyocell cellulose".

According to certain embodiments, the spinning dope may include an aqueous solution of N-methylmorpholine-N-oxide (NMMO). Taking into consideration degree of dissolution of cellulose and process temperature, the aqueous solution may include, for example, a weight ratio of 80 to 95 of N-methylmorpholine-N-oxide and a weight ratio of 5 to 20 of water.

According to certain embodiments, the content of alpha-cellulose in the cellulose or cellulose pulp may be 85 to 97 wt% with respect to 100 wt% of the total cellulose and/or cellulose pulp.

In some embodiments, the content of hemicellulose in the cellulose or cellulose pulp may be 1 wt% to 15 wt% with respect to 100 wt% of the total cellulose. By controlling the content of hemicellulose within the above range, stable physical properties (e.g., hardness or suction resistance implementation) and processability of the lyocell material can be more easily secured.

Additionally, in some embodiments of the present application, the degree of polymerization (DPw) of the cellulose may be 600 to 1700. The polymerization degree may refer to the number of repeating units and/or monomeric units of the components (cellulose, hemicellulose, etc.) contained in the cellulose pulp. In particular, as used in this application, the term "polymerization degree" may refer to the number of monomeric units and/or repeating units in a macromolecule or polymer or oligomer molecule. The polymerization degree (DPw) may be given by DPw = Mn/M0 wherein Mn is the number-average molecular weight of the macromolecule or polymer or oligomer molecule and M0 is the molecular weight of the monomeric unit.

In the spinning step, the shape of a spinneret for discharging the spinning dope is not particularly limited. For example, a donut-shaped spinneret may be used.

The nozzle temperature, specifically, spinning temperature of a spinneret may be appropriately selected by those skilled in the art. Considering that the viscosity of the spinning dope may vary depending on the spinning temperature to result in poor discharging, the spinning temperature may be, for example, 100°C or lower to 120°C or lower, or 100°C or lower to 110°C or lower.

In some embodiments, the step of spinning the spinning dope may be performed under controlled spinning conditions so that the single fineness of a filament is 1.67 dtex to 8.89 dtex (1.5 denier to 8.0 denier) or less. For example, at least one spinning condition of the discharge amount and spinning speed of the spinning dope may be appropriately controlled so that the single fineness of the filament included in the lyocell material satisfies 1.67 to 8.89 dtex (1.5 to 8.0 denier). In this case, the single fineness of a filament refers to the fineness of a single monofilament separated from a multifilament, as already described above.

The upper limit of the single fineness of the filament may be, for example, 8.33 dtex (7.5 denier) or less, 7.78 dtex (7.0 denier) or less, 7.22 dtex (6.5 denier) or less, 6.67 dtex (6.0 denier) or less, 6.11 dtex (5.5 denier) or less, 5.56 dtex (5.0 denier) or less, 5.00 dtex (4.5 denier) or less, 3.89 dtex (3.5 denier) or less, 3.33 dtex (3.0 denier) or less, or 2.78 dtex (2.5 denier) or less. Further, the lower limit of the single fineness thereof may be, for example, 2.22 dtex (2.0 denier) or more, 2.78 dtex (2.5 denier) or more, 3.33 dtex (3.0 denier) or more, 3.89 dtex (3.5 denier) or more, 4.44 dtex (4.0 denier) or more, 5.00 dtex (4.5 denier) or more, 5.56 dtex (5.0 denier) or more, 6.11 dtex (5.5 denier) or more, 6.67 dtex (6.0 denier) or more, 7.22 dtex (6.5 denier) or more, or 7.78 dtex (7.0 denier) or more. When the above range is satisfied, it may be more advantageous in implementing the stable suction resistance of a filter for smoking articles and ensuring the processibility of a filter for smoking articles.

The spinning dope discharged through the spinneret may undergo a coagulating process to be described later.

### <(b) Coagulating and multifilament obtaining step>

In this step, the spun lyocell spinning dope may be coagulated, and lyocell multifilaments may be obtained.

For the coagulation, a method in which the spinning dope comes into contact with air and/or a coagulation liquid may be used.

For example, the coagulation may include a first coagulation step of supplying cooling air to the spun lyocell dope; and a second coagulation step of coagulating the first-coagulated spinning dope by adding the same to a coagulation liquid.

According to the coagulation step, the lyocell dope discharged from the spinneret may be first coagulated in the space (air gap section) between the spinneret and a coagulation tank. This air gap section may be supplied with cooling air from an air-cooling unit located inside the spinneret to the inside to outside of the spinneret. In addition, the first coagulation may be achieved by the so-called air quenching method or means known in the related field.

For example, the upper temperature limit of the cooling air used for the first coagulation may be, for example, 15 °C or less. For example, the cooling air may be air having a temperature of 14 °C or less, 13 °C or less, 12 °C or less, 11 °C or less, or 10 °C or less. When the temperature is exceeded, the coagulation of the spinning dope by air may not be sufficient, and the spinning-related processability may not be good.

The lower temperature limit of the cooling air may be determined in consideration of spinning processability and/or cross-sectional uniformity of a filament. For example, when the temperature of the cooling air is lower than 4°C, the surface of the spinneret may cool, the surface of the filament may become uneven, and the spinning processability may also deteriorate. In consideration of this, the temperature of the cooling air may be, for example, 5 °C or more, 6 °C or more, 7 °C or more, 8 °C or more, or 9 °C or more.

The degree to which the cooling air is supplied may be controlled in consideration of sufficient coagulation, spinning processability, and influence on the physical properties of the filament. For example, the cooling air may be supplied to the discharged spinning dope at an air flow rate of 70 to 400 Nm³/h. For example, the air flow rate may be 100 Nm³/h or more, 150 Nm³/h or more, 200 Nm³/h or more or 250 Nm³/h or more, and the upper limit of the air flow rate may be, for example, 350 Nm³/h or less, 300 Nm³/h or less, 250 Nm³/h or less, 200 Nm³/h or less or 150 Nm³/h or less.

After the first coagulation step, the cooled spinning dope may be supplied to a coagulation tank or bath containing a coagulation liquid (second coagulation step). For appropriate coagulation to proceed, the temperature of the coagulation liquid may be, for example, 30 °C or less or 25 °C or less. Further, the temperature of the coagulation liquid may be, for example, 10 °C or more, 15 °C or more, or 20 °C or more. When the temperature is maintained, a coagulation rate may be appropriately maintained.

The type of the coagulation liquid for the second coagulation as described above is not particularly limited. For example, the coagulation liquid may include at least one of water and N-methylmorpholine-N-oxide (NMMO).

Although not particularly limited, when the coagulation liquid includes water and NMMO, based on 100 wt% of the total weight of the coagulation liquid, the content of water in the coagulation liquid may be 60 to 90 wt%, and the content of NMMO in the coagulation liquid may be 10 to 40 wt%. Alternatively, the coagulation liquid may include 70 to 80 wt% of water and 20 to 30 wt% of NMMO based on 100 wt% of the total weight of the coagulation liquid. The concentration of this coagulation liquid may be controlled to be maintained during the manufacturing process using sensors, etc.

### <(c) Washing step>

If necessary, the lyocell multifilament may be washed after the above-described coagulation and multifilament obtaining step. NMMO and/or other impurities remaining in the filament may be removed by this washing.

The method of performing the washing is not particularly limited. For example, the washing may be performed by introducing the coagulated lyocell multifilaments into a washing tank using a towing roller. Alternatively, the washing may be performed by spraying a washing liquid during the procedure of moving to the next step by a towing roller.

The components of the washing liquid is not particularly limited. For example, the washing liquid may include water, and may further include known additives.

Further, in consideration of reuse after washing, etc., the washing liquid may be used at a temperature of 100 °C or lower.

### <(d) Oil treatment step>

If necessary, a step of treating the lyocell multifilaments with an oil may be performed. This process is a process of applying the above-described oil to the surface of a filament. Through the oil treatment, friction applied to the filament may be reduced, and crimps may be formed well in the crimp application step to be described later. When the oil treatment is performed twice or more as described below, it may be called first oil treatment and second oil treatment depending on the order.

Although not particularly limited, the oil treatment may be performed by immersing the lyocell multifilament in a bath filled with the oil so that the lyocell multifilaments are completely immersed in the oil. Alternatively, the oil may be treated by spraying an oil liquid during the procedure of moving to the next step by a towing roller.

In order to ensure that the amount of the oil applied to the lyocell multifilament after the oil treatment as described above is constant, an additional step may be performed in which a roll or the like positioned before and/or after the oil treatment step squeezes out the oil from the surface of the lyocell multifilament.

For example, the oil treatment may be performed such that the content of the oil (OPU: oil pick up ratio (weight %)) is 1.0 weight % or more based on 100 wt % of the at least oil-treated lyocell multifilament. In this case, the at least oil-treated lyocell multifilament may be, for example, a lyocell multifilament to which first oil treatment has been applied, a lyocell multifilament to which first oil treatment and second oil treatment (refer to the description below) have been applied, or a lyocell multifilament to which a binder to be described below has been applied together with the above-described oil treatment. Further, the lyocell multifilament treated with an oil and/or a binder as described above may be a lyocell multifilament to which crimps are applied.

For example, the content of the oil in the at least oil-treated lyocell multifilament may be 0.5 wt% or more, 1.0 wt% or more, 1.5 wt% or more, 2.0 wt% or more, 2.5 wt% or more, 3.0 wt% or more, specifically, 3.5 wt% or more, 4.0 wt% or more, 4.2 wt% or more, 4.5 wt% or more, 5.0 wt% or more, 5.5 wt% or more, 6.0 wt% or more, 6.5 wt% or more, 7.0 wt% or more, 7.5 wt% or more, 8.0 wt% or more, 8.5 wt% or more, 9.0 wt% or more or 9.5 wt% or more, based on 100 wt% of the total weight of the at least oil-treated lyocell multifilament. Further, the upper limit thereof may be, for example, 20.0 wt% or less, 18.0 wt% or less, 17.0 wt% or less, 16.0 wt% or less, 15.0 wt% or less, 14.5 wt% or less, 14.0 wt% or less, 13.5 wt% or less, 13.0 wt% or less, 12.5 wt% or less, 12.0 wt% or less, 11.5 wt% or less, 11.0 wt% or less, 10.5 wt% or less, 10 wt% or less, 9.5 wt% or less, 9.0 wt% or less, 8.5 wt% or less, 8.0 wt% or less, 7.8 wt%, or 7.6 wt% or less, based on 100 wt% of the total weight of the at least oil-treated lyocell multifilament. In this case, the above content may refer to a dry weight after a solvent (e.g., water) or liquid component that may be included in the oil has evaporated.

When the above-described oil is treated within the above content range, the hydrophilic properties of the lyocell material can be supplemented.

In some embodiments, drying of the oil may be performed after the above-described oil treatment.

In some embodiments of the present application, one or more of the above-described steps may be controlled so that the single fineness of filaments forming the lyocell multifilament may be 1.67 to 8.89 dtex (1.5 to 8.0 denier). The single fineness of the filament refers to a fineness of a single monofilament separated from a multifilament, as described above.

The upper limit of the single fineness of the filament may be, for example, 8.33 dtex (7.5 denier) or less, 7.78 dtex (7.0 denier) or less, 7.22 dtex (6.5 denier) or less, 6.67 dtex (6.0 denier) or less, 6.11 dtex (5.5 denier) or less, 5.56 dtex (5.0 denier) or less, 5.00 dtex (4.5 denier) or less, 3.89 dtex (3.5 denier) or less, 3.33 dtex (3.0 denier) or less, or 2.78 dtex (2.5 denier) or less. Further, the lower limit of the single fineness thereof may be 2.22 dtex (2.0 denier) or more, 2.78 dtex (2.5 denier) or more, 3.33 dtex (3.0 denier) or more, 3.89 dtex (3.5 denier) or more, 4.44 dtex (4.0 denier) or more, 5.00 dtex (4.5 denier) or more, 5.56 dtex (5.0 denier) or more, 6.11 dtex (5.5 denier) or more, 6.67 dtex (6.0 denier) or more, 7.22 dtex (6.5 denier) or more, or 7.78 dtex (7.0 denier) or more. Satisfying the above range may be more advantageous in implementing stable suction resistance of a filter for smoking articles and ensuring processability of a filter for smoking articles.

Although not particularly limited, the step controlled to ensure the above-described single fineness range may be the above-described spinning step. Alternatively, the above-described spinning, coagulation, washing and oil treatment step may all be controlled to ensure the above-described single fineness range.

### <(e) Crimp application step>

The crimp application step is a pstep of applying pressure to the oil-treated lyocell multifilament through steam and/or a press roller to obtain a crimped multifilament, preferably, a crimped tow. The crimp application step may be referred to as a crimping step.

Through the crimping, lyocell multifilaments may be imparted with waves, and fibers may have bulky characteristics. According to some embodiments, the crimping may be performed using a known crimping device, such as one including a stuffer box and/or a steam box, and the usable crimping device is not particularly limited as long as it is a device capable of applying one or more of the pressures to be described below.

For example, the crimp application step may be performed by first supplying steam to the lyocell multifilament to preheat and swell the lyocell multifilament and then pressing the lyocell multifilament with a press roller to form wrinkles in the lyocell multifilament. In this case, a steam box may be used for steam supply, and this steam box may be located at the front end of the crimping device.

For example, the crimp application step may be performed in a manner in which pressurization of the lyocell multifilament by a press roller and steam supply are performed simultaneously.

For example, the crimp application step may be performed by first supplying steam to the lyocell multifilament to preheat and swell the lyocell multifilament and then simultaneously applying pressure and steam to the lyocell multifilament by a press roller.

For example, the crimp application process may be performed by applying steam of 0.98 to 19.61 N/cm² (0.1 to 2.0 kgf/cm²) to the lyocell multifilament before introducing it into the crimping device (for example, press roller).

For example, steam of 1.96 N/cm² (0.2 kgf/cm²) or more, 2.94 N/cm² (0.3 kgf/cm²) or more, 3.92 N/cm² (0.4 kgf/cm²) or more, 4.90 N/cm² (0.5 kgf/cm²) or more or 5.88 N/cm² (0.6 kgf/cm²) or more may be supplied by the steam box. Further, steam of 14.71 N/cm² (1.5 kgf/cm²) or less, 13.73 N/cm² (1.4 kgf/cm²) or less, 12.75 N/cm² (1.3 kgf/cm²) or less, 11.77 N/cm² (1.2 kgf/cm²) or less, 10.79 N/cm² (1.1 kgf/cm²) or less, or 9.81 N/cm² (1.0 kgf/cm²) or less may be supplied. When the steam supply or pressure is below the above range, crimps may not be formed easily. Further, when the steam supply or pressure exceeds the above range, the flexibility of the filament increases to apply excessive crimps within the crimping device, and thus the filament may not pass through the crimping device.

For example, the crimp application step may be performed by pressing the lyocell multifilament with a press roller to form wrinkles in the lyocell multifilament. Further, steam supply may not be performed prior to pressurization, steam supply may not be performed simultaneously with pressurization, or steam supply may not be performed both prior to pressurization and simultaneously with pressurization.

For example, the crimp application step may be performed by applying a pressure of 14.71 to 39.23 N/cm² (1.5 to 4.0 kgf/cm²) to the lyocell multifilament introduced into the crimping device using a press roller.

For example, a pressure of 15.69 N/cm²(1.6 kgf/cm²) or more, 16.67 N/cm²(1.7 kgf/cm²) or more, 17.65 N/cm²(1.8 kgf/cm²) or more, 18.63 N/cm²(1.9 kgf/cm²) or more, 19.61 N/cm²(2.0 kgf/cm²) or more, 20.60 N/cm²(2.1 kgf/cm²) or more, 21.58 N/cm²(2.2 kgf/cm²) or more, 22.56 N/cm²(2.3 kgf/cm²) or more, 23.54 N/cm²(2.4 kgf/cm²) or more, or 24.52 N/cm²(2.5 kgf/cm²) or more may be applied to the lyocell multifilament through the press roller. Further, 38.25 N/cm²(3.9 kgf/cm²) or less, 37.27 N/cm²(3.8 kgf/cm²) or less, 36.29 N/cm²(3.7 kgf/cm²) or less, 35.31 N/cm²(3.6 kgf/cm²) or less, 34.33 N/cm²(3.5 kgf/cm²) or less, 33.35 N/cm²(3.4 kgf/cm²) or less, 32.37 N/cm²(3.3 kgf/cm²) or less, 31.39 N/cm²(3.2 kgf/cm²) or less, 30.41 N/cm²(3.1 kgf/cm²) or less, 29.42 N/cm²(3.0 kgf/cm²) or less, 28.44 N/cm²(2.9 kgf/cm²) or less, 27.46 N/cm² (2.8 kgf/cm²) or less, 26.48 N/cm² (2.7 kgf/cm²) or less, 25.50 N/cm² (2.6 kgf/cm²) or less, or 24.52 N/cm² (2.5 kgf/cm²) or less may be applied to the lyocell multifilament by the press roller.

When the pressure of the press roller is below the above range, the desired number of crimps may not be formed sufficiently. Further, when the pressure of the press roller exceeds the above range, pressing force may be too strong, so that the filament may not be smoothly introduced into the crimping device or may not pass through the stuffer box. Wrinkles may be formed in the lyocell multifilament by the press roller providing the above pressure.

For example, a pressure of 0.98 to 19.61 N/cm² (0.1 to 2 kgf/cm²) may be applied to the lyocell multifilament using an upper plate. Further, the upper plate may apply pressure to the lyocell multifilament when the lyocell multifilament passes through the press roller or is passing through the press roller.

For example, the pressure applied by the upper plate may be 1.96 N/cm² (0.2 kgf/cm²) or more, 2.94 N/cm² (0.3 kgf/cm²) or more, 3.92 N/cm² (0.4 kgf/cm²) or more, or 4.90 N/cm² (0.5 kgf/cm²) or more. Further, a pressure of 14.71 N/cm² (1.5 kgf/cm²) or less, 13.73 N/cm² (1.4 kgf/cm²) or less, 12.75 N/cm² (1.3 kgf/cm²) or less, 11.77 N/cm² (1.2 kgf/cm²) or less, 10.79 N/cm² (1.1 kgf/cm²) or less, or 9.81 N/cm² (1.0 kgf/cm²) or less may be applied by the upper plate.

Furthermore, when the pressure of the upper plate, serving to move up and down to provide uniform crimps after passing through the press roller, is less than 0.98 N/cm² (0.1 kgf/cm²), the upper plate cannot be fixed due to the pressure inside the stuffer box, thereby causing the tow to stay in the stuffer box for a long time to prevent the continuity of a process from being maintained. When the pressure of the upper plate exceeds 19.61 N/cm² (2 kgf/cm²), steam cannot be easily discharged inside the stuffer box, thereby causing the shape of crimps to become irregular.

For example, in the crimp application step, a doctor blade applying a preset pressure to the lyocell multifilament may be used. The doctor blade controls the residence time of the filaments introduced into the crimper, stuffer box, thereby contributing to the control of the number of crimps. This doctor blade may be located in the path of the lyocell multifilament pressed by the roller and then discharged at the roller pressure point.

For example, the crimp application step may be performed by applying a pressure of 0.98 to 19.61 N/cm² (0.1 to 2.0 kgf/cm²) to the lyocell multifilament passing through the roller of the crimping device using the doctor blade.

For example, the pressure applied by the doctor blade may be 1.96 N/cm² (0.2 kgf/cm²) or more, 2.94 N/cm² (0.3 kgf/cm²) or more, 3.92 N/cm² (0.4 kgf/cm²) or more, or 4.90 N/cm² (0.5 kgf/cm²) or more. Further, a pressure of 14.71 N/cm² (1.5 kgf/cm²) or less, 13.73 N/cm² (1.4 kgf/cm²) or less, 12.75 N/cm² (1.3 kgf/cm²) or less, 11.77 N/cm² (1.2 kgf/cm²) or less, 10.79 N/cm² (1.1 kgf/cm²) or less, or 9.81 N/cm² (1.0 kgf/cm²) or less may be applied by the doctor blade.

For example, the crimp application step may be performed at a temperature in the range of 120°C to 250°C. When the temperature is too low, the shape stabilization effect of crimps is not good, and when the temperature is too high, the concentration of oil in the stuffer box increases, thus making it difficult to form crimps. Therefore, considering the above-described steam pressure or the like, the temperature may be, for example, appropriately controlled in a range of 130°C or higher, 140°C or higher, or 150°C or higher, and 200°C or lower, 180°C or lower, or 160°C or lower.

### <(f) Binder treatment step>

In an example, the method may further include a step of treating the oil-treated lyocell multifilamet or the lyocell multifilament obtained by the crimp application step with a binder.

When a filter for smoking articles is manufactured using a lyocell material (e.g., lyocell tow), a binder may be used additionally. The binder may increase the hardness of a filter for smoking articles including a lyocell material, thereby preventing a filter from being caught during a filter manufacturing process or a cigarette manufacturing process.

The binder treatment step can include coating a lyocell material with a binder, the method is not particularly limited. For example, the oil treatment may be carried out by immersing the lyocell multifilaments in a bath filled with a binder (or a binder solution) so that the lyocell multifilaments are completely immersed in the binder. Alternatively, binder coating on the lyocell multifilament may be achieved by injecting (or spraying) a binder (or a binder solution) through a nozzle.

Since the types and components of available binders are as described above, a detailed description thereof will be omitted.

For example, the binder (or binder solution) may further include a solvent in addition to the above-described components. Examples of the solvent may include, but are not limited to, water, ethanol, propylene glycol, and/or glycerin. In some embodiments, the solvent is selected from the group consisting of water, ethanol, propylene glycol, glycerin, or a combination thereof. When the binder (or binder solution) includes a solvent, the content of the solvent may be, for example, about 20 to 80 wt% or about 40 to 60 wt% based on 100 wt% of the total weight of the binder (or binder solution).

The binder treatment may be performed at a level that can achieve the purpose of the above-described binder treatment. For example, the binder treatment may be performed so that the content of the binder satisfies a range of 20 wt% or less, for example, 8 to 15 wt%, based on 100 wt% of the oil and binder-treated lyocell multifilament. In this case, the content may refer to a dry weight after the solvent or liquid component that may be included in the binder has evaporated.

After the lyocell multifilament is coated with the binder, drying of the binder may be performed. Although drying temperature is not particularly limited, for example, drying may be performed at room temperature (about 10 °C to 35 °C).

### <(g) Other steps>

After crimp application, appropriate post-treatment may be additionally performed.

In an example, second oil treatment (g1) may be additionally performed. The second oil treatment may provide more flexibility to a lyocell tow. The second oil treatment may be performed in the same manner as or in accordance with (d) the above-described oil treatment step.

For example, the second oil treatment may be performed by applying an oil to the lyocell tow that has undergone a process using a crimping device. This treatment may be advantageously utilized in various steps performed during the manufacturing of filters for smoking articles. For example, the second oil treatment may allow fibers and filters to be easily spread by air during a spreading step, while also restricting the breakage of fibers during a stretching process.

The above-described second oil treatment may be performed before or after the binder treatment. Alternatively, the second oil treatment may be performed regardless of the binder treatment.

Even in cases where the above-described second oil treatment is performed, a second oil treatment step may be performed so that the content of oil or OPU in the material satisfies the above-described range.

For example, drying treatment (g2) may be performed additionally. The drying may be carried out, for example, at a temperature ranging from 100 °C to 130 °C. The drying treatment method or process is not particularly limited, and known technologies may be used. For example, this drying treatment may be achieved by applying hot air to the lyocell tow or passing the tow through or leaving the tow in a temperature-controlled room for a certain period of time.

In an aspect, the present disclosure provides a lyocell material obtained by a method for manufacturing a lyocell material as described above.

In an aspect, the present disclosure provides a lyocell material obtainable by a method for manufacturing a lyocell material as described above.

### [Smoking articles]

Although not particularly limited, the lyocell material manufactured by the above method may be included in a smoking article. Smoking articles may be aerosol-generating articles. An aerosol-generating article may include an aerosol-generating material or an aerosol-forming substrate.

For example, a lyocell material may be included in a combustible cigarette. Further, the lyocell material, for example, may be included in a heating cigarette, and the heating cigarette may be used in conjunction with an aerosol generating device (not shown).

For example, when a smoking article is used as a heating smoking article, the smoking article may be inserted separately into the aerosol generating device. Here, the aerosol generating device includes a receiving groove capable of receiving an aerosol generating article, and, in addition, may include a heater for heating the aerosol generating article so as to generate an aerosol, a control unit for generally controlling the operation of the aerosol generating device, a battery for providing power used for operating the aerosol generating device, and a detector for recognizing that the aerosol generating article has been inserted into the aerosol generating device.

The smoking article may include a tobacco medium unit, a filter for the smoking article, and a wrapper, wherein the filter for the smoking article may be located at one end of the tobacco medium unit, for example at the rear end or front end of the tobacco medium unit. The tobacco medium unit and the filter for the smoking article may each include a single segment, or may each independently include a plurality of segments.

The tobacco medium unit includes a tobacco material, and the tobacco material includes nicotine. Further, the tobacco medium unit may additionally include one or more excipients.

The excipients may include a binder, a filler, and other additives. For example, a tobacco medium included in the tobacco medium unit may be manufactured in the form of granules including a tobacco material, an excipient, etc.

For example, a filler may be additionally included to maintain the shape, strength and mass of the tobacco medium unit constant. For example, the lyocell material may be included in the tobacco medium unit. Further, the lyocell material may be used as a filler.

The wrapper may be subdivided into a cigarette paper wrapping the tobacco medium unit, a filter wrapping paper wrapping the filter, and a tipping wrapper combining the tobacco medium unit and the filter.

### [Filter for smoking articles]

A lyocell material may be used in a filter for smoking articles. The lyocell material may be a lyocell tow. In an example, the lyocell tow includes a lyocell multifilament to which crimps are applied.

According to an aspect, the present application relates to a filter for smoking articles. The filter for smoking article includes a lyocell material, and the lyocell material may be the same as that described above. Further, the filter for smoking articles may include a lyocell tow, and the lyocell tow may be the same as that described above.

Further, the lyocell material may include the oil in an amount of 0.1 wt% or more with respect to 100 wt% of the total weight of the lyocell material. Besides, the description of the oil component and content according to an embodiment of the present application is the same as those described above.

For example, the single fineness of filaments forming the lyocell multifilament may be 1.5 to 8.0 denier. The specific values are the same as those described above.

For example, the lyocell multifilament to which crimps are applied may be a lyocell material having a total fineness of 15,000 to 55,000 denier, and, preferably, may be a lyocell tow. The specific values are the same as those described above.

For example, the lyocell multifilament to which crimps are applied may have crimps of 3.94 to 19.69 per cm (10 to 50 per inch). Specific values are the same as those described above.

For example, the filter for smoking articles may further include a binder on the surface of the lyocell multifilament to which crimps are applied or between the lyocell multifilament to which crimps are applied. The binder may increase the hardness of a filter for smoking articles manufactured from tow, thereby preventing a filter from being caught during a filter manufacturing process or a cigarette manufacturing process. The description of the types, components and contents of available binders is the same as those described above.

For example, the filter for smoking articles may further include a wrapping paper (referred to as wrapper paper, filter paper or filter wrapping paper). For example, the wrapping paper may be a porous paper or non-porous paper capable of wrapping the above-described lyocell tow and maintaining the shape of a filter (e.g., a column or cylinder).

In certain embodiments of the present application, the filter for smoking articles may have a preset shape and size.

For example, the filter may have a rod shape. For example, the filter for smoking articles may have a cylindrical shape.

Further, the filter may have a length of, for example, 10 mm to 50 mm. For example, the length of the filter may have a lower limit of 15 mm or more, 20 mm or more, 25 mm or more, 30 mm or more, 35 mm or more, 40 mm or more, or 45 mm or more, and may have an upper limit of 45 mm or less, 40 mm or less, 35 mm or less, 30 mm or less, 25 mm or less, 20 mm or less, or 15 mm or less.

In certain embodiments of the present application, the filter having the above length may have a circular cross-section, and the circular cross-section may be a circumference of 10 mm to 40 mm. For example, the circumference of the filter may have a lower limit of 15 mm or more, 20 mm or more, 25 mm or more, 30 mm or more, or 35 mm or more, and may have an upper limit of 35 mm or less, 30 mm or less, 25 mm or less, 20 mm or less, or 15 mm or less.

For example, the filter for smoking articles may include a lyocell tow and a filter wrapping paper. Since the description of the lyocell tow and the filter wrapping paper is the same as that described above, it will be omitted.

The wrapping paper may be a porous paper or non-porous paper capable of wrapping the above-described lyocell tow and maintaining the shape of a filter (e.g., a column or cylinder).

For example, when a porous wrapping paper is used, the wrapping paper may have a porosity of 10 to 50,000 CU (Coresta Unit). Coresta Unit may be defined as a volume flow rate (cm³min⁻¹) of air passing through 1 cm² of a substrate sample (i.e. porous wrapping paper) at a pressure difference of 1 kPa. The lower limit of the porosity of the wrapping paper may be, for example, 1000 CU or more, 5000 CU or more, 10000 CU or more, 15000 CU or more, 20000 CU or more, 25000 CU or more, 30000 CU or more, 35000 CU or more, 40000 CU or more, or 45000 CU or more, and the upper limit thereof may be, for example, 45000 CU or less, 40000 CU or less, 35000 CU or less, 30000 CU or less, 25000 CU or less, or 20000 CU or less. In some embodiments of the present application, the wrapping paper may have a porosity within a range of 22,000 to 26,000 CU or 23,000 to 25,000 CU.

For example, the basis weight of the wrapping paper may be 15 to 60 g/cm². The lower limit of the basis weight of the wrapping paper may be, for example, 20 g/cm² or more, 25 g/cm² or more, 30 g/cm² or more, 35 g/cm² or more, 40 g/cm² or more, 45 g/cm² or more, 50 g/cm² or more, or 55 g/cm² or more, and the upper limit thereof may be, for example, 55 g/cm² or less, 50 g/cm² or less, 45 g/cm² or less, 40 g/cm² or less, 35 g/cm² or less, 30 g/cm² or less, 25 g/cm² or less, or 20 g/cm² or less. In some embodiments of the present application, the wrapping paper may have a basis weight of 16 g/cm² or more, 17 g/cm² or more, 18 g/cm² or more, 19 g/cm² or more, 20 g/cm² or more, or 21 g/cm² or more, and 25 g/cm² or less, 24 g/cm² or less, 23 g/cm² or less, 22 g/cm² or less, or 21 g/cm² or less.

Although not particularly limited, the weight of the rod-shaped filter may be 50 mg or more. The weight of the filter may have, for example, a lower limit of 100 mg or more, 150 mg or more, or 200 mg or more, and may have an upper limit of 500 mg or less, 450 mg or less, 400 mg or less, 350 mg or less, 300 mg or less, 250 mg or less, or 200 mg or less.

Since descriptions of other filters for smoking articles and materials included therein are the same as those described above, they will be omitted.

### [Method of manufacturing filter for smoking articles]

For example, the present application relates to a method of manufacturing a filter for smoking articles. This method is a method of manufacturing the above-described filter for lyocell smoking articles, and may be a method including a method of manufacturing the above-described lyocell material.

With regard to the method of manufacturing a filter for smoking articles, residual steps except for the process of manufacturing the filter are the same as those described for the above-described lyocell material, and therefore, a description thereof will be omitted. Besides, any description that overlaps with those described above will also be omitted.

The process of manufacturing a filter may be appropriately performed by those skilled in the art according to a known method. For example, a filter may be manufactured by forming a wrapping paper filled with a lyocell material into a rod shape. Alternatively, a filter may be manufactured by cutting a filter paper filled with a lyocell material having a rod shape to an appropriate length. A description of the wrapping paper is as the same as that described above.

Although not particularly limited, prior to filling a filter paper with a lyocell material, opening of the lyocell material or treatment with a plasticizer may be additionally performed. The surface area of the lyocell material may be increased by opening the lyocell material. For example, opening of the lyocell material may be performed by applying an external force in a length direction, width direction, and/or thickness direction.

Preferably, the lyocell material used in manufacturing a filter for smoking articles may be a lyocell tow.

Although not particularly limited, the filter for smoking articles may additionally include known cellulose acetate multifilaments at a level that does not hinder the purpose of the present disclosure. Cellulose acetate multifilaments may be blended with lyocell multifilaments. Cellulose acetate multifilaments may be included in a segment distinct from the segment including lyocell multifilaments.

### Advantageous Effects of Invention

According to the present application, there are provided a lyocell material for a filter of smoking articles that can replace commercialized cellulose acetate (CA), and a filter for smoking articles including the same. Specifically, the filter characteristics and processibility of a filter for smoking articles can be harmoniously improved by including a lyocell material satisfying a preset filtration index.

### Mode for the Invention

Hereinafter, the operation and effects of the disclosure will be described in more detail through specific examples of the disclosure. However, this is presented as an example of the disclosure and the scope of the disclosure is not limited thereto in any way.

A lyocell material was prepared through the same process as those described in the following preparation example. Any conditions not specifically mentioned were made within the scope of the above description.

### [Preparation Example]

Cellulose pulp having an alpha-cellulose content of 93.9% and a degree of polymerization (DPw) of 820 was mixed with an NMMO/H₂O solvent having a propyl gallate content of 0.01 wt% to prepare a spinning dope for manufacturing a tow with a concentration of 11 wt%. Then, while maintaining a spinning temperature at 110°C in a spinning nozzle, a discharge amount and a spinning rate were appropriately adjusted, and the spinning dope was spun.

The filament-phase spinning dope discharged from the spinning nozzle was supplied through an air gap section to a coagulation liquid (a coagulation liquid having a concentration of 75 wt% water and 25 wt% NMMO and a temperature of about 25°C) in a coagulation tank. In this case, cooling air in the air gap section first coagulates the spinning dope at a temperature of 8 °C and an air flow rate of 200 N m'/h. Further, the concentration of the coagulation liquid was continuously monitored using a sensor and a refractometer.

Then, the coagulated lyocell filaments were washed. Specifically, filaments were introduced into a towing roller, and NMMO remaining in the filaments was removed by a washing liquid sprayed from a washing device. Then, first oil treatment was performed by immersing the washed filaments into a bath designed to have a preset oil concentration.

In the lyocell material having undergone the first oil treatment, the filaments were treated with a pressure of 29.42 N/cm² (3 kgf/cm²) by a nip roll installed in the discharge unit of the bath, and were introduced into a crimping machine to provide wrinkles. Specifically, the pressure of a press roller was set to 24.52 N/cm² (2.5 kgf/cm²), and the pressure of a doctor blade was set to 4.90 N/cm² (0.5 kgf/cm²) to prepare a lyocell tow. The tow passed through a continuous drying device set to 120°C to obtain a dried tow product.

The prepared tow has a single fineness of 2.22 to 3.89 dtex (2.0 to 3.5 denier), a total fineness of 3,333 to 5,000 tex (30,000 to 45,000 denier), and a crimp number of 5.91 to 23.62 ea/cm (15 to 60 ea/inch).

### Examples 1 to 6

Filters for smoking articles were manufactured using the lyocell material prepared in the above preparation example, and the concentration of a first oil solution and the temperature of the first oil solution were as shown in Table 1.

. Each of the filters for smoking articles had a rod shape. The circumference of each of the filters for smoking articles was 24.2 mm, and the radius of each of the filters was 3.85 mm. In addition, the filling degree, number of crimps, and filtration index of the lyocell material included in each of the filters for smoking articles were as shown in Table 1 below.

### Comparative Examples 1 to 4

Filters for smoking articles were manufactured using the lyocell material prepared in the above preparation example, and the concentration of a first oil solution and the temperature of the first oil solution were as shown in Table 1.

Each of the filters for smoking articles had a rod shape. The circumference of each of the filters for smoking articles was 24.2 mm, and the radius of each of the filters was 3.85 mm. In addition, the filling degree, number of crimps, and filtration index of the lyocell material included in each of the filters for smoking articles were as shown in Table 1 below.

### [Evaluation Example]

### <Experiment 1: Evaluation of filtration index>

Filtration indices were evaluated with respect to the filters for smoking articles according to Examples 1 to 6 and Comparative Examples 1 to 4. The number of crimps was calculated from the lyocell materials collected from the filters for smoking articles.

Specifically, prior to measurement, samples collected from the respective lyocell materials were left and stabilized for 24 hours under conditions of temperature 20±2°C and humidity 65±4%. Thereafter, the number of crimps was measured from each sample using a single fiber property evaluation device (Favimat). Each sample was mounted on a dedicated jig with a length (gauge length) of 10 to 30 mm, and the initial load during measurement was 0.05 g/de, and the crimp sensitivity during measurement was 0.01 mm.

Additionally, the radius of the filter used to evaluate filling degree was 3.85 mm, the length of the filter was 108 mm, and the volume of the filter was 46.6 cm³.

The filling degree of the lyocell material was calculated by dividing an actually measured weight of the lyocell material per unit volume of the filter for smoking articles by a theoretical weight of the lyocell material per unit volume of the filter for smoking articles and multiplying this value by one hundred. The theoretical weight was calculated using the density of the lyocell material and the volume of the filter for smoking articles, and the value obtained by dividing the theoretical weight by the volume of the filter was 0.749 g/cm³. The actually measured weight was measured from the lyocell material included in each filter for smoking articles, and is expressed in weight per filter rod (mg/rod). The measured weight of the lyocell material per unit volume is the same as a weight per volume in Table 1 below.

The weights, weights per length, and weights per volume of the filters for smoking articles according to Examples 1 to 6 and Comparative Examples 1 to 4 are as shown in Table 1 below.

**[Table 1]**

| | | First oil solution concentration (wt%) | First oil solution temperature (°C) | Roller speed ratio of towing roller during last washing | Actually measured weight (mg/rod) | Weight per volume (g/cm³) |
|---|---|---|---|---|---|---|
| Ex a m pl e | 1 | 6.00 | 60.0 | 1.05 | 840 | 0.1669 |
| | 2 | 6.00 | 80.0 | 1.10 | 858 | 0.1705 |
| | 3 | 6.00 | 20.0 | 1.10 | 862 | 0.1713 |
| | 4 | 6.00 | 60.0 | 1.15 | 885 | 0.1758 |
| | 5 | 10.00 | 60.0 | 1.05 | 848 | 0.1685 |
| | 6 | 2.00 | 60.0 | 1.05 | 851 | 0.1691 |
| C o m pa rat iv e Ex a m pl e | 1 | 6.00 | 80.0 | 0.95 | 382 | 0.0759 |
| | 2 | 10.00 | 110.0 | 1.05 | 812 | 0.1613 |
| | 3 | 6.00 | 70.0 | 1.20 | 425 | 0.0844 |
| | 4 | 1.00 | 20.0 | 1.10 | 842 | 0.1673 |

Referring to Preparation Example and Table 1, in the manufacturing of Examples 1 to 6 and Comparative Examples 1 to 4, the first oil treatment conditions and the weight of the lyocell material are delicately controlled. As a result, the filtration indices of the lyocell material and the filter for smoking articles, the filter including the same, are finely controlled, as will be described below.

The crimp number and filling degree of the filters for smoking articles according to Examples 1 to 6 and Comparative Examples 1 to 4 were measured and calculated. Additionally, the filtration indices of each example and each comparative example were calculated based on the number of crimps, the filling degree, and the following Equation 1. The calculation results are shown in Table 2 below. $Filtration index = filling degree * number of crimps$

**[Table 2]**

| | | Number of crimps (ea/cm) | Filling degree (%) | Filtration index |
|---|---|---|---|---|
| Example | 1 | 13.78 | 22.28 | 779.9 |
| | 2 | 11.42 | 22.76 | 660.0 |
| | 3 | 14.96 | 22.87 | 868.9 |
| | 4 | 13.78 | 23.48 | 821.6 |
| | 5 | 8.66 | 22.49 | 494.9 |
| | 6 | 16.93 | 22.57 | 970.7 |
| Comparative Example | 1 | 12.20 | 10.13 | 314.1 |
| | 2 | 5.12 | 21.54 | 280.0 |
| | 3 | 9.84 | 11.27 | 281.8 |
| | 4 | 20.87 | 22.33 | 1183.8 |

Referring to Table 2, it was confirmed that each of the filters for smoking articles of Examples 1 to 6 had a filtration index of 400 to 1000. On the other hand, it was confirmed that each of the filters for smoking articles according to Comparative Examples 1 to 4 had a filtration index of less than 400 or more than 1000.

### <Experiment 2: Evaluation of filters for smoking articles>

The suction resistance and processibility of the filters for smoking articles according to Examples 1 to 6 and Comparative Examples 1 to 4 were evaluated. The suction resistance was measured according to KS H ISO 6565. The processibility was evaluated as good when the manufacturing of a lyocell material is possible continuously and the manufacturing of filters for smoking articles, each filter including the lyocell material, is also possible continuously. The processibility was evaluated as poor when the manufacturing of the lyocell material and/or the manufacturing of the filters for smoking articles are restricted.

In the case of Comparative Example 4, the manufacturing process of the filter for smoking articles could not be continuously performed due to the bursting of filter paper.

The evaluation results for the suction resistance and processibility of the filters for smoking articles according to Examples 1 to 6 and Comparative Examples 1 to 4 are as shown in Table 3 below.

**[Table 3]**

| | | Suction resistance (mmH₂O) | Processibility |
|---|---|---|---|
| Example | 1 | 720 | good |
| | 2 | 690 | good |
| | 3 | 775 | good |
| | 4 | 765 | good |
| | 5 | 610 | good |
| | 6 | 780 | good |
| Comparative | 1 | 263 | good |
| Example | 2 | 218 | good |
| | 3 | 215 | good |
| | 4 | manufacturing of filter is restricted | |

Referring to Table 3, it was confirmed that the filters for smoking articles of Examples 1 to 6 provide a suction resistance of 600 mmH₂O or more even though they include the lyocell material, which is an environmentally friendly material. It can be evaluated that the suction resistance as described above is comparable to that of a filter for smoking articles, the filter including a conventional cellulose acetate material.

On the other hand, it was confirmed that the filters for smoking articles of Comparative Examples 1 to 3 provide a suction resistance of 300 mmH₂O or less. Accordingly, it is confirmed that the filter for smoking articles according to each example can provide improved filtering performance compared to the filter for smoking articles according to each comparative example.
Meanwhile, the manufacturing process of the filter for smoking articles according to Comparative Example 4 could not be continuously performed due to the bursting of filter wrapping paper, and the evaluation of the suction resistance could not be performed.

## Claims

1. A lyocell material comprising: a lyocell multifilament to which crimps are applied,
wherein the lyocell material has a filtration index of 400 to 1000, represented by Equation 1 below: $Filtration index = filling degree \times number of crimps$
wherein in Equation 1,
the filling degree is a value obtained by dividing an actually measured weight of the lyocell material per unit volume by a theoretical weight of the lyocell material per unit volume and multiplying this value by one hundred.

2. The lyocell material of claim 1,
wherein in Equation 1,
the filling degree is a value obtained by dividing an actually measured weight of the lyocell material per unit volume of a filter for smoking articles by a theoretical weight of the lyocell material per unit volume of the filter for smoking articles and multiplying this value by one hundred.

3. The lyocell material of claim 1,
wherein the filling degree is 15% to 30%.

4. The lyocell material of claim 1,
wherein the number of crimps is 10 ea/inch to 60 ea/inch.

5. The lyocell material of claim 1,
wherein the filling degree is 15% to 30%, and the number of crimps is 15 ea/inch to 60 ea/inch.

6. The lyocell material of claim 1,
wherein the filling degree is 21% to 24%, and the number of crimps is 20 ea/inch to 45 ea/inch.

7. The lyocell material of claim 1,
wherein the lyocell multifilament includes one or more monofilaments, and at least one of the monofilaments has a non-circular cross-section.

8. The lyocell material of claim 1,
wherein the lyocell multifilament includes one or more monofilaments, and all of the monofilaments each have a non-circular cross-section.

9. The lyocell material of claim 1,
wherein the lyocell multifilament has a single fineness of 1.5 denier to 8.0 denier.

10. The lyocell material of claim 1,
wherein the lyocell material has a total fineness of 15,000 to 55,000.

11. The lyocell material of claim 1,
wherein the lyocell material is a lyocell tow.

12. The lyocell material of claim 1,
wherein the lyocell material is used for a filter for smoking articles.

13. The lyocell material of claim 1,
wherein the lyocell material is not used for tire cord nor for cloth.

14. A filter for smoking articles, the filter comprising the lyocell material of any one of claims 1 to 13.

15. A smoking article comprising the filter for smoking articles of claim 14.
